

E. H. ANGIER.

GUMMED PAPER AND METHOD OF MANUFACTURING THE SAME.

APPLICATION FILED AUG. 16, 1919.

1,357,020.

Patented Oct. 26, 1920.

**Fig. 1.**



**Fig. 2.**



**Inventor:**

*Edward H. Angier,  
by George Barth, James Henry  
Altiss.*

# UNITED STATES PATENT OFFICE.

EDWARD H. ANGIER, OF FRAMINGHAM, MASSACHUSETTS.

## GUMMED PAPER AND METHOD OF MANUFACTURING THE SAME.

1,357,020.

Specification of Letters Patent. Patented Oct. 26, 1920.

Application filed August 16, 1919. Serial No. 317,907.

To all whom it may concern:

Be it known that I, EDWARD H. ANGIER, a citizen of the United States, and resident of Framingham, in the county of Middlesex and Commonwealth of Massachusetts, have invented an Improvement in Gummed Paper and Methods of Manufacturing the Same, of which the following description, in connection with the accompanying drawings, is a specification, like characters on the drawings representing like parts.

This invention relates to gummed paper and to methods of manufacturing the same. The purpose is to provide an article of superior flexibility and strength and also one which is not liable to objectionable curling.

My invention will best be understood by reference to the following description taken in connection with the accompanying drawings wherein:

Figure 1 is a diagrammatic view illustrating one specific method of preparing gummed paper, and

Fig. 2 is a plan view of a portion of a gummed strip.

My invention may perhaps be best understood if I first describe one particular method of preparing the paper as illustrated diagrammatically in Fig. 1. As there shown I take crinkled or craped paper 3, the crinklings of which preferably extend transversely to the grain of the paper. The crinkled paper may conveniently be prepared from finished paper in the manner described in the Arkell Patent 790,021. The crinkled strip of paper 3 is then preferably stretched as indicated by the arrows in Fig. 1 to reduce the crinklings to a considerable degree and one side thereof is then coated with a suitable adhesive gum as indicated diagrammatically by the moistening roll 5. In Fig. 2 the gum coating is indicated by the stippling 7 on the vertical portion of the paper and as shown the crinklings or crapings are apparent on both sides. Though not necessarily limited thereto I preferably prepare the paper as herein described by first craping it and then gumming it and also by extending the crapings by stretching the paper. While the finished product in its preferred form has a certain elasticity and stretch due to the residual expansibility of the crapings, the latter are considerably reduced and the effect may conveniently be rather that of a superior softness and pliability than that of elas-

ticity although a certain elasticity remains in the paper which permits it to adapt itself to more or less irregular surfaces.

Gummed paper prepared in this manner appears to have the gum coating broken up more or less along the lines of the crinklings. It is of a comparatively soft cloth-like texture in spite of the dried coating of gum and this flexibility is obviously highly desirable for many purposes. When used in the form of a tape for application to box corners or the like the crinkling provides a certain transverse reinforcement, strengthening the tape transversely and also transversely of the natural grain of the paper. A great difficulty has been found with gummed paper because of its tendency to curl when dried, particularly in a direction transverse to the grain. I find that this difficulty is obviated to a considerable extent with the paper described.

While I am not prepared to state definitely the theoretical cause of the properties of the paper which as I have empirically demonstrated do exist, I advance the following possible explanations: First it may be that the coating of gum as it dries and shrinks ebbs, as it were, from the minute elevations formed by the crinklings and into the corresponding hollows. The continuity of the gum coating is thus broken up or its thickness is in such a way varied that while the gummed surface is continuous for adhesive purposes, it does not exert a curling pull on the paper. It is further possible that the contraction of the gum in drying draws elastically upon the crinklings of the paper until the paper backing is in a state of equilibrium although still lying flat. Since curling has hereto been most marked transversely to the grain of the paper which is ordinarily longitudinal of the strip or web, it is probable that such curling has taken place because the paper bent more easily in that direction instead of along the grain where curling is resisted by the fibers. It is possible that the transverse crinklings provide a sort of artificial grain giving a reinforcement similar to that given to iron by corrugating it, which resists such curling.

It may be noted that in whatever manner the effect is obtained there is no weakening of the paper. It has been customary to attempt to prevent gummed paper from curling by breaking up the gum coating after

it has dried in place. This has necessitated a sharp bending or pounding of the paper likely to weaken the same just as paper is weakened by folding and creasing. As contrasted thereto a given length of paper made as here described is probably actually stronger in a transverse direction and, as already pointed out, this is of considerable advantage for many purposes to which such adhesive paper is adapted.

It will be understood that by gum I refer to suitable material which under ordinary conditions is dry and hard but which may readily be softened and rendered adhesive by moistening.

Having thus described one preferred embodiment of my invention by way of illustration, what I claim as new and desire to secure by Letters Patent is:—

20 Claims:

1. The method of manufacturing gummed paper which comprises:—crinkling the pa-

per, stretching the crinkled paper and applying a gum coating.

2. The method of manufacturing gummed 25 paper which comprises first crinkling the paper and then applying a coating of gum thereto.

3. Gummed paper wherein the paper base is provided with minute crinkles substantially transverse to the grain. 30

4. Gummed paper having a crinkled paper base and a gum coating the uniformity of which is interrupted by the crinklings.

5. Gummed paper having a paper base 35 generally uniform but provided with minute irregularities in substantial equilibrium with the gum coating.

6. Crinkled paper having a dried gum coating on a face thereof. 40

In testimony whereof I have signed my name to this specification.

EDWARD H. ANGIER.